

## UNITED STATES PATENT OFFICE.

WILLIAM S. CALCOTT, OF PENNSGROVE, NEW JERSEY, ASSIGNOR TO E. I. DU PONT DE NEMOURS & COMPANY, OF WILMINGTON, DELAWARE, A CORPORATION OF DELAWARE.

## PROCESS OF MAKING A LEAD-ALKALI-METAL ALLOY.

No Drawing.

Application filed October 23, 1922. Serial No. 596,517.

*To all whom it may concern:*

Be it known that I, WILLIAM S. CALCOTT, a citizen of the United States, and a resident of Pennsgrove, in the county of Salem 5 and State of New Jersey, have invented a certain new and useful Process of Making a Lead-Alkali-Metal Alloy, of which the following is a specification.

This invention relates to a process of 10 making an alloy of lead and sodium, and comprises heating together sodium and lead to form a homogeneous molten mass while preventing reactive gas, such as air, from coming in contact with the lead or sodium 15 by maintaining over the upper surface of said mass a liquid layer or film of a material which will not contaminate the alloy, and whose melting point is substantially lower than that of said alloy.

20 The composition of the particular alloy with which my invention is chiefly concerned corresponds to the formula  $PbNa_2$ . The melting point of this alloy is about 400° C.

25 The material which I have found to be especially advantageous for use as a protective layer for the molten lead-sodium alloy, is a mixture of sodium hydroxide and potassium hydroxide, and preferably the eutectic mixture, that is 60% caustic potash and 40% caustic soda.

My invention may be illustrated in greater detail by the following example:

In a crucible provided with a carbon 35 dioxide ( $CO_2$ ) inlet and supply are placed 13 parts of lead and 3 parts of sodium. The air is then swept out with a current of  $CO_2$ , and heat applied. When the temperature of the sodium reaches 150° C., the lead begins to dissolve with a vigorous evolution 40 of heat. When the temperature reaches 200° C., 10 parts of mixed caustic (60% KOH, 40% NaOH) are added. The sodium by this time has dissolved sufficient lead 45 so that the density is greater than that of the caustic, which consequently floats on the surface and protects the alloy from oxidation. The mass is then maintained in a molten condition until it has become homogeneous. As the melting point of the mixed 50 caustic is only 175° C., while that of the alloy is 400° C., the caustic serves as an efficient protective layer till long after the al-

loy has become solid, in which state it is relatively non-reactive.

The layer of caustic may be removed by pouring it off in the molten condition after the alloy has cooled sufficiently to solidify.

Although I prefer to use the eutectic mixture of the hydroxides of sodium and potassium, it will be understood that various other mixtures may be used without departing from my invention.

The procedure described above may also be used in the manufacture of alloys of lead 65 and some other alkali-metal such as potassium.

I claim:

1. The process of making an alloy of lead and an alkali-metal, which comprises heating the two metals together to form a molten mass, and excluding oxygen therefrom by maintaining over the upper surface of the molten alloy a liquid layer of a substance which will not contaminate said alloy, 75 and which has a boiling point above, and a melting point substantially below, the temperature of said molten alloy.

2. A process of the kind set forth in claim 1 in which the liquid layer comprises a mixture of the hydroxides of sodium and potassium.

3. A process of the kind set forth in claim 1 in which the liquid layer comprises the eutectic mixture of the hydroxides of sodium and potassium.

4. The process of making an alloy of lead and sodium, which comprises heating the two metals together with exclusion of oxygen to form a molten mass, and continuing 90 to exclude oxygen therefrom by maintaining over the upper surface of the molten alloy a liquid layer of a substance which will not contaminate said alloy, and which has a boiling point above, and a melting point 95 substantially below, the temperature of said molten alloy.

5. A process of the kind set forth in claim 4 in which the liquid layer comprises a mixture of the hydroxides of sodium and potassium.

6. A process of the kind set forth in claim 4 in which the liquid layer comprises the eutectic mixture of the hydroxides of sodium and potassium.

7. The process of making a lead-sodium

55

70

75

80

85

90

95

100

105

alloy of approximately the composition  $PbNa_2$ , which comprises heating 130 parts of lead with about 30 parts of sodium in an atmosphere of carbon dioxide until the mass <sup>5</sup> has a temperature of about  $200^\circ C.$ , then adding a mixture comprising essentially 6 parts of potassium hydroxide and 4 parts of sodium hydroxide, increasing the tem-

perature of the mass until a homogeneous molten alloy is formed with a layer of the <sup>10</sup> molten caustic mixture covering the alloy, and then allowing the molten alloy to solidify before removing the caustic mixture.

In testimony whereof I affix my signature.

WILLIAM S. CALCOTT.